

## UNITED STATES PATENT OFFICE

RICHARD H. STRATTON, OF BERKELEY, CALIFORNIA, ASSIGNOR TO ATLAS POWDER COMPANY, OF WILMINGTON, DELAWARE, A CORPORATION OF DELAWARE

## EXPLOSIVE COMPOSITION

No Drawing.

Application filed February 27, 1931. Serial No. 518,916.

This invention relates to explosive compositions and particularly to the type known as dynamites and to the use of novel carbonaceous combustible materials in the preparation of such explosive compositions. The chief object of the invention is to provide novel, economical, solid, carbonaceous combustible ingredients, having relatively high densities and relatively low absorbencies for the liquid explosive ingredients. Further objects will become apparent with the following description of my invention, such as, for example, (1) the provision of carbonaceous ingredients for dynamite with little or no desensitizing effects on the explosive ingredients in contact therewith and (2) the provision of carbonaceous ingredients for dynamite having domestic sources of supply.

So-called dynamites usually comprise one or more solid and/or liquid explosive compounds, such as nitroglycerine, nitroglycol, nitropolyglycerine, dinitrotoluene, trinitrotoluene, nitrocotton, nitro-starch, and the like; one or more oxygen carrying salts, such as ammonium nitrate, sodium nitrate and the like and one or more fuels, such as sulphur, starch, charcoal, wood meal, vegetable ivory meal, bagasse pith and the like.

In formulating explosives of the dynamite type, it is necessary,—in order to obtain the proper efficiency and desired characteristics,—to so balance the above three types of ingredients that the desired strengths, densities, velocities of detonations, sensitivities to detonation, stabilities, oxygen balances, water resistances and degrees of cohesiveness will be attained. The proper choice of a fuel or fuels, for a dynamite composition, is accordingly of very great importance. Some of the more important considerations, involved with the choosing of a fuel for a dynamite are described herewith. First, the fuel must be such that it will not induce instability in the explosive compound or compounds, with which it is to be in direct con-

tact; second, it must be such that it will not desensitize the explosive compound or compounds after extended contact; third, it must be such that it will hold the liquid constituents by absorption and thereby prevent exudation or leakage, without having so much excess absorption that the explosive will be rendered too insensitive to be detonated by ordinary explosive initiators and to propagate efficiently; fourth, it must have proper density or specific gravity to impart the required density to the ultimate explosive for the desired density of loading; fifth, it must have proper particle size and be of such physical structure as to not only impart the desired velocity of detonation but also to provide proper aeration in the ultimate explosive, when mixed with the other ingredients; sixth, its color must be as light as possible to impart a good appearance to the ultimate explosive; seventh, its chemical composition must be such as to provide the evolution of a large volume of gaseous products of combustion, resulting in good strength effects by the ultimate explosive; and eighth, it must require an amount of oxygen to complete its combustion, which can be provided by limited amounts of economical oxygen carriers, in order to assure the evolution of minimum amounts of poisonous gases in the products of detonation of the ultimate explosive.

From the above, it will be seen that there are several requisites which are common to all types of dynamite fuels, whereas other requisites are dependent upon the particular types of ultimate explosive compositions involved. The chief requisites of the latter type are those involving the density, the fineness (particle size) and the absorbency of the dynamite fuel. For example, a dynamite of the straight nitroglycerine type requires a highly absorptive fuel, such as wood pulp, sawdust and the like, in order that the liquid nitroglycerine will be held by absorption entirely, whereas a low density permissible ex-

plosive, having a relatively small nitroglycerine content, requires a low density fuel, with as low absorbency as possible, such as bagasse pith and the like.

5 Likewise, it is just as important to have a satisfactory fuel, having a relatively high density and a relatively low absorptive capacity for liquid explosives, for use in controlling the density and absorption of many 10 types of dynamite. For certain types of dynamite, such as, for example, low strength gelatin dynamites, practically no cellular absorption is required at all; the nitroglycerine being merely held by gelatinization with 15 nitrocotton and by adherence to the surfaces of the non-absorbent particles of the fuels and oxygen carriers. For certain other types of dynamite, a limited amount of absorption is required, examples of which are 20 the low strength nitroglycerine dynamites, the intermediate strengths of gelatin dynamite and nearly all of the so-called ammonium nitrate dynamites. In this case, just enough absorption must be provided to prevent 25 the exudation or leakage of the liquid ingredients; an excess of absorption being avoided by the use of the relatively dense, and relatively poor absorbent type of fuel.

Heretofore, vegetable ivory meal has been 30 extensively and almost exclusively used to fulfill the functions of a relatively dense and poorly absorbent fuel. It is derived from the vegetable ivory nut, which is imported into the United States from tropical countries, 35 chiefly for the purpose of making buttons; the scrap and waste material from the button manufacture being reduced to comminuted form for use as the dynamite-fuel. The availability of this material is accordingly 40 directly and entirely dependent upon the operation of the vegetable ivory button factories, since the high cost of importing the vegetable ivory nuts would prohibit their importation for use in dynamite alone. In 45 view of this situation, it is quite evident that it would be advantageous to have a similar type of dynamite fuel, the source of supply of which is domestic as well as more stable and assured.

50 After extensive research and the study and trial of many types of carbonaceous materials from various sources, I have discovered a material which not only fulfills all of the general or common requisites for a dynamite fuel, but also fulfills all of the special requisites, peculiar to a fuel having relatively high density and low absorbency. This material is comminuted almond hulls, which I have also referred to as "almond hull pulp".

55 Comminuted almond hulls or almond hull pulp has the advantages, over vegetable ivory meal, of being a domestically grown product, and of being a by-product from an edible nut. For these reasons, its supply is more stable; 60 less subject to the normal fluctuations of the

manufacturing industry than that of vegetable ivory meal, and more economical.

Extensive tests have also shown almond hull pulp to induce no objectionable destabilizing or desensitizing effects on such liquid explosive as nitroglycerine and nitroglycol. It has also been found to require exactly the same amount of oxygen, per unit weight, to complete its combustion, as ordinary wood pulp. Its ash content (about 2%) is also well within the normal range for commonly used dynamite fuels and its ultimate analysis shows the proportions of carbon and hydrogen to be quite comparable with various carbonaceous materials, which have long been used successfully as dynamite fuels. Satisfactory explosive strength results also confirm the satisfactory gas producing quality for almond hull pulp, when used in liberal quantities in dynamite. Its light ochre color is also quite satisfactory for a dynamite fuel of its type.

Although the density of almond hull pulp is not quite as high as that of vegetable ivory meal, it is sufficiently high to be used almost as a direct substitute for vegetable ivory meal. Experiments have shown that the same density may be retained in a dynamite composition by replacing a small amount of a comparatively light and highly absorbent fuel, in addition to the replacement of all of the vegetable ivory meal, in the original composition. By using this procedure, the almond hull pulp not only has the advantage of entirely replacing all of the vegetable ivory meal but also may have the advantage of replacing a portion of a more costly absorbent fuel as well. In fact, it has been determined that the slightly lower density of almond hull pulp, as compared with vegetable ivory meal, entails a corresponding slight increase in absorbency, which permits of the substitution procedure, described above, with the retention of proper absorption as well as density in the ultimate dynamite composition.

The following table shows examples of dynamite compositions, which serve to illustrate the application of the substitution procedure described above.

|                                                                 | 40% dynamite<br>(amm. nit. type) |          | 35% gelatin<br>dynamite |          | 120 |
|-----------------------------------------------------------------|----------------------------------|----------|-------------------------|----------|-----|
|                                                                 | Per cent                         | Per cent | Per cent                | Per cent |     |
| Liquid explosive.....                                           | 17.5                             | 17.5     | 29.1                    | 29.1     |     |
| Solid explosive.....                                            | 4.5                              | 4.5      | 0.4                     | 0.4      |     |
| Nitrocotton.....                                                |                                  |          |                         |          |     |
| Nitrate of soda.....                                            | 41.0                             | 41.0     | 54.7                    | 54.7     |     |
| Nitrate of ammonia.....                                         | 25.0                             | 25.0     |                         |          |     |
| Wood pulp.....                                                  | 5.0                              | 4.0      | 1.3                     | 0.3      |     |
| Vegetable ivory meal.....                                       | 6.0                              |          | 5.0                     |          |     |
| Almond hull pulp.....                                           |                                  | 7.0      |                         | 6.0      |     |
| Flour.....                                                      |                                  |          | 5.0                     | 5.0      | 125 |
| Sulphur.....                                                    |                                  |          | 3.5                     | 3.5      |     |
| Ant-acid.....                                                   | 1.0                              | 1.0      | 1.0                     | 1.0      |     |
| Number of $1\frac{1}{4} \times 8''$ ctgs. per 50<br>pounds..... | 113                              | 113      | 83.2                    | 84.5     |     |
| Sensitivity to detonation.....                                  | 16''                             | 16''     | 8''                     | 9''      |     |
| Velocity of detonation—MPS.....                                 | 3033                             | 3126     | 2387                    | 2477     | 130 |

Additional examples of dynamite compositions, using almond hull pulp as a fuel, are shown in the following table:

|                      | Per cent | Per cent | Per cent |
|----------------------|----------|----------|----------|
| 5 Nitroglycerine     | 22.5     | 19.5     | 10.5     |
| TNT                  | 2.3      | 3.5      |          |
| Nitrocotton          | .3       |          |          |
| Ammonium nitrate     | 5.0      |          | 75.0     |
| Ammonium perchlorate |          | 5.0      |          |
| Nitrate of soda      | 54.8     | 52.0     | 5.0      |
| Almond hull pulp     | 4.6      | 14.0     | 5.5      |
| Starch               | 5.0      |          |          |
| 10 Sulphur           | 5.0      |          |          |
| Ant-acid             | 5.0      | 1.0      | .5       |
| Sawdust              | .5       |          |          |
| Bagasse pith         |          | 5.0      | 3.5      |

To those versed in the art of formulating dynamite compositions, it is well known that the particle size or fineness of a carbonaceous dynamite fuel plays an important part in affecting various properties of the ultimate dynamite composition, examples of which are 15 the velocity of detonation, the sensitiveness, the cohesiveness, the water resistance and the density. It is for this reason that various degrees in the fineness of such fuels as vegetable ivory meal have been employed to control such properties in a dynamite composition, as exemplified above.

The degree of fineness of almond hull pulp, I have discovered, has very similar effects on these properties as that of vegetable ivory meal. In fact, almond hull pulp has an additional advantage over vegetable ivory meal, because of the fact that vegetable ivory scrap often includes a large proportion of relatively fine particles, whereas almond hulls are usually obtainable in comparatively coarse form; thereby permitting a larger proportion of relatively coarse almond hull pulp to be derived from almond hulls, if desired, than the proportion of relatively coarse vegetable ivory meal, derivable from the average run of ivory nut scrap.

Another advantage arising from the use of almond hull pulp, particularly in relatively coarse form, in contradistinction to the use of other forms of ground nut shells, is the ease and completeness with which the meats may be separated from the hulls. I am aware of the fact that it has heretofore been proposed to use other forms of nuts, such, for example, as walnuts and pecans. However, the use of almond hulls presents marked advantages over any other nut shells or hulls which have ever been proposed for the purpose stated. For example, the patent to Barab, No. 1,280,634 discloses the very expensive and troublesome methods which have to be resorted to to separate the shells of such nuts as walnuts and pecans from the adherent meats which are found clinging to them when they are received by the explosives manufacturers. Further, walnut and pecan nut shells are much more oily than almond hulls, and oily materials are desensitizers and must be avoided in the relationship in which I find almond hulls to be of the greatest utility,

namely, as a substitute for ground vegetable ivory. Further, almond hulls present a difference in kind even with respect to the scarce and expensive ground vegetable ivory for which I propose to substitute it, in that it is 70 decidedly less gritty than the ground vegetable ivory and it is well recognized that grittiness of dynamite particles involves an increased hazard in use as well as in manufacture. Almond hull pulp possesses the desired 75 low absorbency or the capacity to retain the nitroglycerine in the form of a surface film rather than as an absorbed constituent without being so compact as to enter into combustion with difficulty. In this respect it is 80 superior to the more expensive ground vegetable ivory and by its use it is possible to make gelatins and low nitroglycerine dynamites with good propagation sensitiveness and very 85 slow development of insensitiveness and inertness of agent.

It should accordingly be clearly understood that my invention is not limited as to the particle size of the almond hull pulp employed as a dynamite fuel, although I prefer it to include no particles, sufficiently large to be held on a screen having a 0.10 inch square opening, for my purpose. While I have found that almond hulls may be suitably reduced to almond hull pulp by means 90 of either an attrition mill or squirrel-cage mill, it is to be understood that my invention is not limited to these types of mills, but that any type of mill, grinder, pulverizer or disintegrator may be used to reduce the almond 95 hulls to almond hull pulp of any fineness desired, without being outside the scope of my invention.

It should also be clearly understood that the almond hull pulp may be substituted for all or part of one or more combustible fuels, in any type of explosive composition and that it may be used either alone or in conjunction with other combustible materials, without departing from my invention, and that the amount of almond hull pulp employed may be varied at will, since I contemplate using up to about 25% of the same. It is also understood that the invention covers the use of almond hull pulp in conjunction with various types of liquid explosive materials, both in their liquid and gelatinized states. As examples of liquid explosives that may be employed, in conjunction with almond hull pulp, I may mention nitroglycerine, tetranitrodiglycerine, glycol dinitrate or oily dinitrotoluene. Various solid explosive materials may be used; for example, crystalline dinitrotoluene, nitrocotton or crystalline tri-nitrotoluene, as well as various oxidizing materials, as for example, inorganic nitrates, ammonium nitrate, chlorates, perchlorates or metallic oxides. Explosive compositions, within the scope of my invention, also may or may not have their flame temperature re-

duced for safety toward the ignition of gases or dusts in mines, in ways well known to those skilled in the art.

To avoid any possible misinterpretation, I  
5 wish it clearly understood that the terms  
commminuted almond hulls and almond hull  
pulp are inclusive of the terms ground al-  
mond shells.

Having described my invention, what I  
10 claim is:

1. A dynamite containing almond hull  
pulp as a combustible ingredient.
2. A gelatin dynamite containing almond  
hull pulp as a combustible ingredient.
- 15 3. A non-gelatinous dynamite containing  
almond hull pulp as a combustible ingredient.
4. A dynamite composition containing  
from one-half of one per cent to twenty-five  
per cent of almond hull pulp as a combustible  
20 ingredient.
5. A dynamite comprising a fuel consist-  
ing of comminuted almond hulls and a liquid  
explosive ingredient for which said almond  
hulls have at least partial absorbent capacity.
- 25 6. A dynamite comprising an oxidizing  
material, comminuted almond hulls and a  
liquid explosive ingredient for which said  
almond hulls have at least a partial absorb-  
ent capacity.
- 30 7. A dynamite comprising an oxidizing  
material, comminuted almond hulls and a  
liquid explosive ingredient for which said  
almond hulls have at least a partial absorb-  
ent capacity, and wherein the almond hulls  
35 have been comminuted to such a degree as to  
pass through a 0.10 inch square opening.
8. A dynamite comprising a carbonaceous  
fuel consisting of almond hull pulp, and  
nitroglycerine.

40 In testimony whereof I, RICHARD H. STRAT-  
TON, affix my signature.

RICHARD H. STRATTON.

45

50

55

60